

Patented Apr. 24, 1923.

1,453,259

# UNITED STATES PATENT OFFICE.

ROBERT JOHN, OF NEW YORK, N. Y.

## PRINTING PLATE AND PROCESS AND COMPOSITION OF MATTER FOR FORMING THE SAME AND PROCESS OF PRINTING.

No Drawing.

Application filed August 16, 1922. Serial No. 532,321.

To all whom it may concern:

Be it known that I, ROBERT JOHN, a citizen of the United States, a resident of the city of New York, in the county of New York and State of New York, have invented certain new and useful Improvements in Printing Plates and Processes of and Compositions of Matter for Forming the Same and Processes of Printing, of which the following is a specification.

My invention relates to printing plates and processes of and compositions of matter for forming the same, and has, among other objects, the following: first, the production of a plate, and particularly a lithographic plate, and more particularly of a plate such as is used in photo-gelatine printing processes, and a process of printing by which plate printing press prints or reproductions may be made of a quality superior to any hitherto known in the art; second, the production of such a plate by which such prints or reproductions may be produced at a speed greatly in excess of any hitherto possible in the art; third, the devising of a process by which a printing plate may be produced with less labor and expense and in a shorter time than has hitherto been possible in the art, and fourth, the production of such a plate which shall reduce the loss of time arising from press stops to a hitherto unattained minimum; and to such ends my invention consists in the improvement in printing plates and processes of and compositions of matter for forming the same and processes of printing hereinafter specified.

My invention is capable of embodiment in many different forms of plates and processes of producing such plates and of printing and by the use of various compositions of matter in such production, and, while I shall choose, for the purpose of illustrating my invention, the best embodiment thereof known to me, such embodiment is to be regarded only as typical and my invention is not to be confined thereto.

The example chosen for illustration is designed for use on a litho-offset printing press. I may use as a base or backing for the plate, thin plates formed of metal, such as aluminum or zinc, ranging in thickness, for example, from .01 to .03 inches, or I may use other materials, such as a sheet of pyroxylin, pyralin, or celluloid for such

purpose. For the illustrative example, a metal plate is chosen, and the first step is to produce a grain or roughness on one side of the plate for the purpose of increasing adherence of the gelatine coat thereto which I next put on it. For this purpose I preferably effect a graining equivalent to that of fine mudground glass, preferring that the grain should be as fine as possible and merely presenting a rough surface. It is to be understood that, as the said graining is simply for the purpose of securing the gelatine coating to the plate, it does not appear in the imprint from the plate and has no effect thereon as would be the case with the grains which are produced on photo-lithographic or offset plates for the purpose of breaking up the continuity of the photographic image.

Having produced a grain upon my plate and thoroughly cleaned it of grit and metallic particles, as by a water spray, I apply the coat of gelatine thereto in any desired manner, as by whirling it with a solution of gelatine. A suitable solution for the purpose may consist of water, 32 ounces, and hard commercial gelatine, 2250 grains, the gelatine having first been soaked in cold water and then brought into solution by raising the temperature to 120° F. The gelatinous solution thus prepared is applied on the center of the grained plate, while the latter is whirling at a rate, say of approximately 20 revolutions per minute, the temperature being preferably maintained at 120° F., under which conditions a proper thickness of coating is obtained. For my purpose I prefer a coating measuring approximately .0008 to .0012 inches in thickness. The plate is preferably permitted to whirl until it is dry.

Having coated my plate and preferably dried it, I preferably subject the gelatine to a hardening agent, such as a bath consisting of alcohol, 32 ounces, and formaldehyde, 40%, 1 ounce, to which the plate is subjected for five minutes. The plate is then preferably again dried as in an enclosed whirler for five minutes and subsequently washed in cold running water for five minutes, when it is again preferably dried, as by whirling. The plate is now ready for the preferably next succeeding operation, which is that of sensitizing. I find that plates thus coated keep indefinitely without deterioration and

I am, therefore, able to coat and harden them in quantities and have a supply always on hand ready for sensitizing.

Having coated and preferably hardened 5 my plate, I sensitize it by a composition which, directly or indirectly, will render the gelatine selectively receptive to a printing medium, such as ink. In the present instance, I sensitize the plate by immersion 10 for two minutes in the following solution:

|                     |     |        |
|---------------------|-----|--------|
| Water               | 16  | ounces |
| Alcohol             | 32  | "      |
| Ammonium bichromate | 450 | grains |

15 after which I dry as by whirling.

The proportions of the ammonium bichromate in such solution may be increased or decreased, according to the result desired and according to the character of the negative to be printed from. In some cases I 20 find it advisable to add a light restraining agent to the sensitizing solution, a typical formula for which would be—

|                     |     |        |
|---------------------|-----|--------|
| Water               | 16  | ounces |
| Alcohol             | 32  | "      |
| Ammonium bichromate | 450 | grains |
| Erythrosine         | 90  | "      |

25 The plate being sensitized, is ready for 30 exposure to light behind a negative (or a positive) and, as in the case of most chromaticized colloids, I find it desirable to effect exposure as soon after sensitizing as possible inasmuch as deterioration soon sets in.

35 If, after having performed the above described steps, I were to wash my plate in cold running water, I would find that those portions of the plate affected by light were harder than those portions unaffected by light. I, however, do not wash the plate at 40 this stage of its preparation as would be done in other processes. While, in my plate, at this stage there is a difference between the light-affected areas and those unaffected 45 by the light, yet that difference is insufficient to enable the plate to receive ink selectively.

Having effected the exposure under the negative, I next proceed with the steps which give it its great selective ink receptivity, as well as its later durability. For 50 this purpose I desire to selectively increase the hardening action which has been started by the light in the chromaticized colloid, and to do so without equally hardening the colloid in its unaffected areas. I preferably 55 use as a hardening agent a substance which, when the excess of such agent is removed, leaves the light-affected portions of the film, and preferably the entire surface of the film, 60 in a dry state. I further prefer to use a hardening agent which also is not absorbed by the film. Therefore, having exposed my plate, and preferably without having washed out the unaltered bichromate, I preferably 65 subject it immediately to a harden-

70 ing agent, such, for instance, as to a bath of grain alcohol of high proof,—preferably 95 per cent. or higher,—or to one of ether or to one of ether and alcohol combined in any desirable proportion. After two minutes of immersion in the said selective hardening bath, I next remove the bichromate from the unaffected parts of the gelatine as by washing the plate for five minutes or more, at the same time removing whatever soluble bichromate may remain in the affected portions. 75

80 Preferably after again washing the plate, I further harden the hardened portions, as by placing the plate in a bath of pure grain alcohol of high proof for two minutes. I find that although the unhardened portions are water-soaked, they are not materially affected by this treatment, since the ammonium salt has been washed out. After 85 this second bath of alcohol I again dry the plate, preferably by whirling, whereupon it is ready for the last step in its preparation—namely, that of heating. This is effected by 90 placing the plate in say, for three minutes, 95 an oven in which, for instance, a temperature of approximately 400° F. is maintained. I find that the effect of the heating is two-fold; first, the heat completes whatever 98 chemical action has been started between the gelatine and bichromate through light exposure and the alcohol, and thereby materially hardens the light-affected areas and 100 brings the plate to a point where there will be no further hardening effect even though the plate be kept for months, since all the 105 chemical action is complete; second, I find that heating as described has the effect of toughening the unaffected portions of the gelatine without materially reducing their 110 water receptiveness, and at the same time increasing the degree of adhesion between the gelatine coating and the grained metal plate. 115

120 When the heating operation is complete, my plate is ready for the press and, when fastened thereto, requires only moistening by water by such means as are to be found on litho and offset presses to be a completed printing plate.

125 When ink is applied to the wet surface of my plate in printing, I find that, in effect, the ink is emulsified with the water and that a very effective printing results therefrom, the ink being so readily deposited on a print, or on a rubber blanket, as in offset printing, and redeposited therefrom upon the print or final support that, not only are prints of high quality obtained, but they are produced at a much greater rate than has ever been done before.

130 My invention, while having some similarities to other printing processes, has marked differences from and advantages over any of them which are known to me. I shall refer

particularly to photo-lithography, photo-offset, and photo-gelatine, or collotype printing processes (which are described in Cassell's Encyclopædia of Photography, Cassell & Co., 1912).

The quality of the prints or reproductions obtainable by my invention in a printing press is markedly superior to those obtainable in that manner by any other process 10 known in the art, including those just referred to, and the rate of production is also much above that possible with such prior art. By my invention forty times as many prints 15 can be made in a given time as with the previous photo-gelatine processes.

In all photo-gelatine processes prior to mine, it has been necessary to form a grain or reticulation in order to create a sufficient selective ink receptivity to attain commercial 20 results, but it is not necessary to use that expedient with my invention. It has also been necessary, prior to my invention, to treat the photo-gelatine plate with a glycerine solution in order to increase said selective 25 ink receptivity. But my plate may be used smooth and grainless, and I employ plain water in moistening it before inking, no glycerine or other agent for swelling the gelatine being required.

30 It is to be noted that in the present example a chromic acid salt is incorporated into my film by first forming the gelatine film on the plate and then afterwards introducing the chromic acid salt by bathing the film in a 35 solution of such salt, and when a film is thus formed, it will not become reticulated even though in the previous drying it had been dried at a temperature which, if the salt had been incorporated with the gelatine while 40 the latter was in solution, would cause reticulation,—namely, a temperature approximating or above 130° F. I can, however, incorporate, the chromic acid salt in the film by introducing it into a solution of the gelatine before the latter is deposited upon the plate to form the film, by evaporation of its 45 solvent, and still obtain a film that is free from reticulation, so long as I do not heat it above 130° F.

50 While the portions of my colloid film which have not been affected by light are so receptive to water that they perfectly reject the ink without the aid of any other expedient than moistening, the portions of the film 55 which have been affected by light and which are to receive the ink to form the image still possess some capacity for absorbing water, and this capacity, in co-operation with the other qualities given to the light affected 60 portions by my said treatment, in some way renders such portions unusually receptive to ink.

Because, therefore, of the fact that I print 65 from a wet ink-receptive surface, while the photo-litho and photo-offset plates are print-

ed with a dry ink-receptive surface, I am able to deposit on the finished print a quantity of color impossible with such processes, and am therefore enabled to print at much greater speeds than their plates permit. Furthermore, I effect a noteworthy saving in 70 press operation through the fact that, while the photo-litho and photo-offset plates have a tendency to oxidize in the air and to lose their water receptivity, which makes necessary, at frequent intervals, a certain operation known as "gumming," my plate cannot oxidize and requires no gumming, and in no way increases the number or duration of 75 press stops. In other words, with my plate, 80 it is not necessary to stop the press for gumming, or for any other operation to renew the selective receptivity of the plate to the ink which forms the print, as such selective 85 receptivity depends only on the presence of the water, and this is automatically renewed after each impression from the plate and without any stoppage of the press.

Referring to the marked superiority in 90 quality of prints and reproductions made according to my invention, as compared with the quality of those made by the three printing processes above mentioned: In the photo-gelatine process, there is of necessity a grain or reticulation, finer or coarser, which 95 is inherent to the formation of the plate. This grain makes it impossible to usefully photograph upon the plate from a half-tone screen negative, or any other negative in which the image is broken up into dots, 100 grains, or particles. My plate being free from grain and reticulation may receive its image either from a continuous tone negative or from a negative made from a half-tone screen or from one in which any manner of dot, grain, or particle is employed.

The plates used in the photo-litho and photo-offset processes must of necessity be made from negatives embodying a dot or grain. On the other hand, my plate, printed 110 on the same press, may be absolutely continuous in tone and free from dot or grain, or, if desired, it may embody a dot or grain, which may be very much finer than any 115 other grain hitherto capable of use in the said process. With my process, I have found it practicable to use dots which were six times as many to the inch as the most that have been used in photo-litho and photo-offset processes, so far as I am aware. For instance, 120 in practice it has been found that a dot averaging 120 to the inch produces the best results in photo-litho and photo-offset printing, and, while dots as fine as 175 to the inch have been employed, they have not been 125 deemed commercially practicable or come into general use. With my plate, however, under commercial conditions I have found it practicable to use a dot as fine as 400 to the 130 inch and a grain as fine as 1200 to the inch.

The degree of fineness of the dot or grain which it is possible to use with my plate is limited only by the ability to produce a screen bearing them. While, in theory, a continuous tone image such as my plate alone is capable of rendering is theoretically desirable, yet, due to inequalities of paper surface and other commercial factors, I find it usually preferable to employ a very fine screen or grain, but it is characteristic of my plate that its wearing qualities and its ability to give continuously perfect reproductions are not influenced, one way or the other, by the fineness of the dot or grain used.

A suitable way in which to form dots upon one of my plates is to form them on the negative, from which the plate is to be printed, in a camera in the manner in which dots are formed in the well-known half-tone process, where the dots are formed by focusing a screen, either regular or irregular, between the lens and the sensitive plate.

A suitable way in which to form grain or reticulation on one of my plates is by printing from a negative made as described in my United States Patent No. 1,374,853, April 12, 1921.

In all reproductive processes, other than mine, wherein a screen, either dot or grain, is used whether in photo-engraving for relief printing or photo-offset or lithography for photographic printing, a number of steps are involved in the process which forbid the use of a dot or grain as fine as that which I can employ. These steps are those intermediate between the exposure of the colloidal bichromated surface to the light and the actual inking of the plate on the press. They involve, for instance, developing away unexposed portions with water and cotton wool, rubbing up with ink or acid resist, etching, re-etching, etc. No matter how careful the manipulations, these operations would change the character or formation of the dot or grain, if one were present as fine as I am able to use, so that much of the result accomplished by exposure to light would be lost when the printing plate was finally inked.

In my process, there is no change in the surface of the plate between its condition when exposed to light and its condition when finally inked to make an impression, and there are no manipulations that can possibly change the size, shape, or character of the dots imprinted by the light. I believe, in fact, that I am the first to produce a printing plate capable of taking ink on a printing press on which the impression is to be formed in which the dots or grains produced by light action are unaltered by manipulations of any kind; such as, reticulation, development, etc., previously mentioned. I further believe that I am the first

to prepare a printing plate wherein the ink image corresponds exactly to the action of the light in the exposure.

A printing plate made according to my invention will receive ink selectively as to its light affection from a roller passed over its surface at a much higher speed than will any other photo-gelatine plate or plate having a colloid film with which I am familiar. With my plate, the ink-applying roller may be passed over its surface at a speed greater than six inches per second.

In my process, as the portions of the plate which are to print the image are moistened with water before ink is applied to them, and are at all times both water-receptive and charged with water, and as, when ink has been applied to such portions, the water and oil do not separate into distinct bodies when heavy pressure is applied between the plate and the paper or rubber blanket upon which the impression is to be made, the water and oil are in an essentially emulsified condition. In the black portions of the print, there are no white areas, as would be the case if the water were as a whole separated from the oil rather than holding the oil in an emulsified condition. Moreover, the ink does not appear to have the power of adhesion to the gelatine surface which it would ordinarily have, a fact which is consistent with its being in an emulsified condition in the water, and I believe this condition explains why my plate will print with so greatly increased a speed. This emulsification of the ink and water I regard as very important and believe it to be a strong factor both in obtaining the relatively great density of color which the plate will print and the high speed with which it will print.

By the term "mechanical inking," as used in the claims, is meant inking by the mere use of a mechanically-operated roller or other device as distinguished from rubbing, stippling with a brush, or rolling by hand, or other manual operation.

By the term "chromic acid salt" it is meant to include every compound of chromium having the property of more or less hardening organic matter under the action of light.

Many modifications of my invention can be made without departing therefrom or from the scope of the claims, and my invention is not limited to the particular embodiment chosen for the purpose of illustration.

Having particularly described my invention, what I claim and desire to secure by Letters Patent is:

1. A printing plate comprising an unreticulated colloid film which is capable of printing after mechanical inking.
2. A printing plate comprising an unreticulated colloid film which is capable of printing after mechanical inking.

- ticulated gelatine film which is capable of printing after mechanical inking.
3. A printing plate comprising a colloid film which is capable of printing after mechanical inking without the use of glycerin or other similar swelling means.
4. A printing plate comprising a gelatine film which is capable of printing after mechanical inking without the use of glycerin or other similar swelling medium.
5. A printing plate comprising a colloid film having dots or grains photographed thereon which in the finished plate are unaltered from the form in which they were originally photographed on such plate.
6. A printing plate comprising a gelatine film having dots or grains photographed thereon which in the finished plate are unaltered from the form in which they were originally photographed on such plate.
7. A printing plate comprising an unreticulated colloid film having ink-receptive portions that are interrupted by relatively very fine dots, or grains, or similar devices.
8. A printing plate comprising an unreticulated gelatine film having ink-receptive portions that are interrupted by relatively very fine dots, or grains, or similar devices.
9. A printing plate comprising a colloid film having ink-receptive portions that are interrupted by dots, grains or similar devices that are photographed thereon.
10. A printing plate comprising a gelatine film having ink-receptive portions that are interrupted by dots, grains or similar devices that are photographed thereon.
11. As an article of manufacture, a photo-gelatine printing plate having the ability to take on ink selectively as to its light affection from an inking roller passed over its surface at a rate exceeding six inches per second.
12. A planographic printing plate capable of receiving ink selectively as to its light affection, from a roller passed over its surface at a speed greater than six inches per second, in which the portions of the plate unaffected by light are composed of a colloid.
13. A planographic printing plate capable of receiving ink selectively as to its light affection, from a roller passed over its surface at a speed greater than six inches per second, which comprises a colloid film, all of the original colloidal material of the film being present in the portions of the finished plate unaffected by light.
14. A printing plate in which the ink-receptive image is composed of an unreticulated colloid that is capable of accepting moisture.
15. A printing plate in which the ink-receptive image is composed of an unreticulated gelatine that is capable of accepting moisture.
16. A planographic printing plate in which the ink-receptive image is composed of a colloid that is free from granular structure and capable of accepting moisture.
17. A planographic printing plate in which the ink-receptive image is composed of a gelatine that is free from granular structure and capable of accepting moisture.
18. A printing plate capable of printing after mechanical inking and comprising an unreticulated colloidal film that is selectively receptive to ink, all of the original colloidal material of the film being present in the finished plate.
19. A printing plate capable of printing after mechanical inking and comprising an unreticulated gelatine film that is selectively receptive to ink, all of the original gelatinous material of the film being present in the finished plate.
20. A printing plate capable of printing after mechanical inking and comprising an unreticulated colloidal film having the image represented by a mere change in the water-receptivity of the corresponding portions of said film.
21. A printing plate capable of printing after mechanical inking and comprising an unreticulated gelatine film having the image represented by a mere change in the water-receptivity of the corresponding portions of said film.
22. A printing plate comprising a colloid film having the image represented thereon by means of dots or grains formed in a camera.
23. A printing plate comprising an unreticulated colloid film having the image represented thereon by means of dots or grains formed in a camera.
24. A printing plate capable of printing after mechanical inking and comprising an unreticulated colloidal film having the image represented by a mere change in the water-receptivity of the corresponding portions of said film and without the removal of any portions of the colloidal material of the film.
25. A printing plate capable of printing after mechanical inking and comprising an unreticulated gelatine film having the image represented by a mere change in the water-receptivity of the corresponding portions of said film and without the removal of any portions of the gelatinous material of the film.
26. A printing plate capable of printing after mechanical inking and comprising a colloid film, in which has been incorporated a chromic acid salt that has been exposed to light, and the hardness of the light-affected portions of which has been increased by the application of other hardening means.
27. A printing plate capable of printing

after mechanical inking and comprising a gelatine film, in which has been incorporated a chromic acid salt that has been exposed to light, and the hardness of the 5 light-affected portions of which has been increased by the application of other hardening means.

28. A printing plate capable of printing after mechanical inking and comprising 10 a colloid film consisting of hardened and relatively unhardened portions, the hardened portions comprising a chromic acid salt, and having been subjected to exposure to light and further subjected to the action 15 of a hardening agency, the relatively unhardened portions remaining relatively unaltered.

29. A printing plate capable of printing after mechanical inking and comprising 20 a gelatine film consisting of hardened and relatively unhardened portions, the hardened portions comprising a chromic acid salt, and having been subjected to exposure to light and further subjected to the action of 25 a hardening agency, the relatively unhardened portions remaining relatively unaltered.

30. A printing plate comprising a colloid film consisting of hardened and relatively 30 unhardened portions, the hardened portions comprising a chromic acid salt and having been subjected to exposure to light and further subjected to the action of alcohol, the relatively unhardened portions remaining 35 relatively unaltered.

31. A printing plate comprising a gelatine film consisting of hardened and relatively unhardened portions, the hardened 40 portions comprising a chromic acid salt and having been subjected to exposure to light and further subjected to the action of grain alcohol, the relatively unhardened portions remaining relatively unaltered.

32. A printing plate comprising a colloid film consisting of hardened and relatively unhardened portions, the hardened portions comprising a chromic acid salt and having 45 been subjected to exposure to light and further subjected to the action of grain alcohol and heating, the relatively unhardened portions remaining relatively unaltered.

33. A printing plate comprising a gelatine film consisting of hardened and relatively unhardened portions, the hardened 55 portions comprising a chromic acid salt and having been subjected to exposure to light and further subjected to the action of grain alcohol and heating, the relatively unhardened portions remaining relatively unaltered.

34. A printing plate comprising a colloid film in which has been incorporated a chromic acid salt that has been exposed to light and the hardness of the light-affected 60 portions of which has been increased by the

use of a hardening agent which, when the excess thereof has been removed, leaves said light-affected portions in a dry state.

35. A printing plate comprising a colloid film in which has been incorporated a 70 chromic acid salt that has been exposed to light and the hardness of the light-affected portions of which has been increased by the use of a hardening agent which, when the excess thereof has been removed, leaves the 75 said film in a dry state.

36. A printing plate comprising a colloid film in which has been incorporated a 80 chromic acid salt that has been exposed to light, and the hardness of the light-affected 85 portions of which has been increased by the use of a hardening agent which is not absorbed by the film.

37. A printing plate comprising a colloid film in which has been incorporated a 85 chromic acid salt that has been exposed to light, and the hardness of the light-affected 90 portions of which has been increased by the application of a hardening agent which is not absorbed by said light-affected portions. 95

38. A printing plate comprising a colloid film in which the parts corresponding to the image are relatively highly receptive to ink when wet with water.

39. A printing plate comprising a gelatine 95 film in which the parts corresponding to the image are relatively highly receptive to ink when wet with water.

40. A printing plate comprising an unreticulated colloid film in which the parts 100 corresponding to the image are receptive to ink when wet with water.

41. A printing plate comprising an unreticulated gelatine film in which the parts 105 corresponding to the image are receptive to ink when wet with water.

42. A printing plate comprising a colloid film having parts corresponding to an image that are receptive to ink, the other portions 110 of said film being capable of continuously repelling ink by the mere application of water.

43. A printing plate comprising a gelatine film having parts corresponding to an 115 image that are receptive to ink, the other portions of said film being capable of continuously repelling ink by the mere application of water.

44. The process of making a printing plate, comprising sensitizing a colloid film with a chromic acid salt, subjecting the same 120 to the selective action of light to form an image, hardening the light-affected areas more than the unaffected areas, and removing the unaffected chromic acid salt.

45. The process of making a printing plate, comprising sensitizing a colloid film with a chromic acid salt, subjecting the same 125 to the selective action of light to form an image, and hardening the light-affected 130

- areas more than the unaffected areas without removing any portion of the colloid.
46. The process of making a printing plate, comprising sensitizing a colloid film with a chromic acid salt, subjecting the same to the selective action of light to form an image, hardening the light-affected areas, removing the unaffected chromic acid salt, and heating the plate.
47. The process of making a printing plate, comprising sensitizing a colloid film with a chromic acid salt, subjecting the same to the selective action of light to form an image, hardening the light-affected areas without removing any portion of the colloid, and heating the plate.
48. The process of making a printing plate comprising sensitizing a gelatine film with a chromic acid salt, subjecting the same to the selective action of light to form an image, hardening the light-affected areas more than the unaffected areas, and removing the unaffected chromic acid salt.
49. The process of making a printing plate comprising sensitizing a gelatine film with a chromic acid salt, subjecting the same to the selective action of light to form an image, and further hardening the light-affected areas more than the unaffected areas without removing any portion of the gelatine.
50. The process of making a printing plate comprising sensitizing a gelatine film with a chromic acid salt, subjecting the same to the selective action of light to form an image, further hardening the light-affected areas, removing the unaffected chromic acid salt, and heating the plate.
51. The process of making a printing plate comprising sensitizing a gelatine film with a chromic acid salt, subjecting the same to the selective action of light to form an image, further hardening the light-affected areas without removing any portion of the gelatine, and heating the plate.
52. The process of making a printing plate comprising forming a colloid film on the plate and sensitizing the film with a chromic acid salt by applying thereto a solution of said salt, exposing said film to a light image and hardening said film.
53. The process of making a printing plate comprising forming on a backing a colloid film that is sensitized by a chromic acid salt and drying said film by a temperature that is not greater than 130° F., exposing said film to a light image and hardening said film.
54. The process of making a printing plate comprising forming a gelatine film on the plate and sensitizing the film with a chromic acid salt by applying thereto a solution of said salt, exposing said film to a light image and hardening said film.
55. The process of making a printing plate comprising forming on a backing a gelatine film rendered sensitive by a chromic acid salt and drying said film by a temperature that is not greater than 130° F., exposing said film to a light image and hardening said film.
56. As a composition of matter, a colloid in which has been incorporated a chromic acid salt, which has been hardened by the action of light, and the hardness of which has been increased by immersion in grain alcohol.
57. As a composition of matter, a colloid in which has been incorporated a chromic acid salt, which has been hardened by the action of light, and the hardness of which has been increased by immersion in grain alcohol and by heating.
58. As a composition of matter, a colloid in which has been incorporated a chromic acid salt, and which has been hardened by light, and the hardness of which has been further increased by the application of a hardening agent.
59. As a composition of matter, a colloid, in which has been incorporated a chromic acid salt and which has been hardened by light, and the hardness of which has been further increased by the application of grain alcohol as a hardening agent.
60. As a composition of matter, a gelatine in which has been incorporated a chromic acid salt, which has been hardened by the action of light, and the hardness of which has been increased by immersion in grain alcohol.
61. As a composition of matter, a gelatine in which has been incorporated a chromic acid salt, which has been hardened by the action of light, and the hardness of which has been increased by immersion in grain alcohol and by heating.
62. As a composition of matter, a gelatine, in which has been incorporated a chromic acid salt and which has been hardened by light, and the hardness of which has been further increased by the application of a hardening agent.
63. As a composition of matter, a gelatine, in which has been incorporated a chromic acid salt, and which has been hardened by light and the hardness of which has been further increased by the application of a grain alcohol as hardening agent.
64. As a composition of matter, a colloid, in which has been incorporated a chromic acid salt some only of which has been hardened by light, and the hardness of which has been further increased by heating both the hardened and unhardened portions of said colloid being present in said composition.
65. As a composition of matter, a gelatine, in which has been incorporated a chromic acid salt some only of which has

been hardened by light, and the hardness of which has been further increased by heating both the hardened and unhardened portions of said gelatine being present in said composition.

66. As a composition of matter, a colloid, in which has been incorporated a chromic acid salt and which has been hardened by light, and the hardness of which has been further increased by the application of a hardening agent and by heating.

67. As a composition of matter, a gelatine, in which has been incorporated a chromic acid salt and which has been hardened by light, and the hardness of which has been further increased by the application of a hardening agent and by heating.

68. In the process of forming a printing plate having a colloid film, the step which comprises hardening the film with formaldehyde before sensitizing it.

69. In the process of forming a printing plate having a colloid film, the step of hardening the film before sensitizing it.

70. In the process of forming a printing plate having a gelatine film, the step of hardening the film before sensitizing it.

71. In the process of forming a printing plate having a colloid film, the step which comprises hardening the film with grain alcohol and formaldehyde before sensitizing it.

72. In the process of forming a printing plate having a gelatine film, the step which comprises hardening the film with grain alcohol and formaldehyde before sensitizing it.

73. The process of making a printing plate comprising coating a backing with gelatine, hardening the gelatine with formaldehyde, sensitizing the gelatine with a chromic acid salt, hardening the light-affected areas by the use of means which will not equally harden the unaffected areas, and then removing the unaffected chromic acid salt from the plate.

74. The process of making a printing plate comprising coating a backing with colloid, hardening the colloid with formaldehyde, sensitizing the colloid with a chromic acid salt, hardening the light-affected areas by the use of means which will not equally harden the unaffected areas, and then removing the unaffected chromic acid salt from the plate.

75. The process of making a printing plate comprising coating a backing with gelatine, hardening the gelatine with formaldehyde, sensitizing the gelatine with a chromic acid salt, applying a light-restraining agent thereto, hardening the light-affected areas by the use of means which will not equally harden the unaffected areas and

then removing the unaffected chromic acid salt from the plate.

76. The process of making a printing plate comprising coating a backing with a colloid, hardening the colloid with formaldehyde, sensitizing the colloid with a chromic acid salt, applying a light-restraining agent thereto, hardening the light-affected areas by the use of means which will not equally harden the unaffected areas and then removing the unaffected chromic acid salt from the plate.

77. The process of making a printing plate comprising coating a backing with gelatine, hardening the gelatine with formaldehyde, sensitizing the gelatine with a chromic acid salt, hardening the light-affected areas by the use of means which will not equally harden the unaffected areas, removing the unaffected chromic acid salt from the plate and then heating said plate.

78. The process of making a printing plate comprising coating a backing with a colloid, hardening the colloid with formaldehyde, sensitizing the colloid with a chromic acid salt, hardening the light-affected areas by the use of means which will not equally harden the unaffected areas, removing the unaffected chromic acid salt from the plate and then heating said plate.

79. The process of making a printing plate comprising coating a backing with gelatine, hardening the gelatine with formaldehyde, sensitizing the gelatine with a chromic acid salt, applying a light-restraining agent thereto, hardening the light-affected areas by the use of means which will not equally harden the unaffected areas, removing the unaffected chromic acid salt from the plate, and then heating said plate.

80. In the process of forming a printing plate having a colloid film, the step which comprises increasing the difference in water-receptivity between those portions of the plate which are more receptive to water than those which are less so.

81. In the process of forming a printing plate having a colloid film, the step which comprises increasing with grain alcohol the difference in water-receptivity between those portions of the plate which are more receptive to water than those which are less so.

82. The process of printing which comprises the application of ink to a wet unreticulated colloidal surface and the printing or transfer of said ink.

83. The process of printing which comprises giving to portions of an unreticulated colloidal surface the capacity when wet to receive ink to form an image, and to other portions of said surface the capacity to repel ink, applying ink to said surface and printing therefrom.

84. The process of printing which com-

prises the application of ink to a wet unreticulated colloidal surface, the transfer of said ink to a rubber blanket, and the transfer of said ink image from said rubber blanket to its final support.

85. The process of printing which comprises forming on a backing a colloid coating, sensitizing said colloid with a chromic acid salt, exposing said colloid to a light image, accentuating the difference in water-receptiveness between the exposed and unexposed portions of the colloid, moistening said plate and applying ink thereto.

86. The process of printing which comprises forming on a backing a colloid coating, sensitizing said colloid with a chromic acid salt, exposing said colloid to a light image, accentuating the difference in water-receptiveness between the exposed and unexposed portions of the colloid by hardening said exposed portions, moistening said plate and applying ink thereto.

87. The process of printing which comprises forming on a backing a gelatine coating sensitizing said gelatine with a chromic acid salt, exposing said gelatine to a light image, accentuating the difference in water-receptiveness between the exposed and unexposed portions of the gelatine by hardening said exposed portions, moistening said plate and applying greasy ink to the less water-receptive areas.

88. The process of printing which comprises forming on a backing a gelatine coating, sensitizing said gelatine with a chromic acid salt, exposing said gelatine to a light image, accentuating the difference in water-receptiveness between the exposed and unexposed portions of the gelatine, moistening said plate and applying ink thereto.

89. The process of printing which comprises forming on a backing a gelatine coating, sensitizing said gelatine with a chromic acid salt, exposing said gelatine to a light image, accentuating the difference in water-receptiveness between the exposed and unexposed portions of the gelatine, moistening said plate and applying ink thereto.

90. The process of printing comprising forming a plate having a colloid film, rendering said film selectively water-receptive according to the image desired, applying only a single ink-repelling medium to said plate and then applying ink to said plate.

91. The process of printing comprising forming a plate having a colloid film, rendering said film selectively water-receptive according to the image desired, applying only water to said plate and then applying ink to said plate.

92. The process of printing which comprises applying ink to a wet surface, emulsifying said ink with water from said wet surface, and printing said ink.

93. The process of printing which comprises applying ink to a wet colloid surface, emulsifying said ink with water from said wet colloid surface, and printing said ink.

94. The process of printing which comprises applying ink to a wet gelatine surface, emulsifying said ink with water from said wet surface, and printing said ink.

95. The process of printing which comprises applying ink to a wet surface, emulsifying said ink with water from said wet surface, depositing said emulsified ink upon a rubber blanket, and redepositing said emulsified ink upon the print or final support.

96. The process of printing which comprises applying ink to a wet colloid surface, emulsifying said ink with water from said wet surface, depositing said emulsified ink upon a rubber blanket, and redepositing said emulsified ink upon the print or final support.

97. The process of printing which comprises applying ink to a wet gelatine surface, emulsifying said ink with water from said wet gelatine surface, depositing said emulsified ink upon a rubber blanket, and redepositing said emulsified ink upon the print or final support.

98. The process of printing which comprises the steps of applying ink to an unreticulated colloidal planographic plate, the image on which has been formed by the action of light and which has remained mechanically unmodified between the step of exposure to light and the said step of applying the ink, and impressing said ink upon a support.

99. The process of making a printing plate comprising forming on a backing a colloid coating, rendered sensitive with a chromic acid salt, exposing the same to a light image, hardening the light-affected areas by means which will not equally harden the unaffected areas, removing the unaffected chromic acid salt from the plate, and heating the plate, and during which process avoiding heating the plate to 130° F. while unaltered chromic acid salt is present in the colloid coating.

100. The process of making a printing plate comprising forming on a backing a gelatine coating rendered sensitive with a chromic acid salt, exposing the same to a light image, hardening the light-affected areas by means which will not equally harden the unaffected areas, removing the unaffected chromic acid salt from the plate, and heating the plate, and during such process avoiding heating the plate to 130° F. while unaltered chromic acid salt is present in the gelatine coating.

101. The process of printing which comprises forming on a backing a gelatine coating, hardening said coating, sensitizing said gelatine with a chromic acid salt, exposing

said gelatine to a light image, then without removing the unaltered portion of said salt, accentuating the difference in water-receptiveness between the exposed and unexposed portions of the gelatine, removing the unaffected portions of said salt from the said gelatine coating hardening said gelatine coating and heating said plate, moistening said plate, applying ink thereto, emulsifying said ink with the said water on said plate and transferring said ink.

102. The process of printing which comprises forming on a backing a colloid coating, hardening said coating, sensitizing said colloid with a chromic acid salt, exposing said colloid to a light image, then without removing the unaltered portion of said salt, accentuating the difference in water-receptiveness between the exposed and unexposed portions of the colloid, removing the unaffected portions of said salt from the said colloid coating hardening said colloid coating and heating said plate, moistening said plate, applying ink thereto, emulsifying said ink with the said water on said plate and transferring said ink.

fected portions of said salt from the said colloid coating, hardening said colloid coating and heating said plate, moistening said plate, applying ink thereto, emulsifying said ink with the said water on said plate and 25 transferring said ink.

103. The process of printing which comprises applying ink to a wet colloid surface; emulsifying said ink with water on said wet surface by pressure, and printing said ink. 30

104. The process of printing which comprises applying ink to a wet gelatine surface; emulsifying said ink with water on said wet surface by pressure, and printing said ink. 35

In testimony that I claim the foregoing, I have hereunto set my hand this 11th day of August, 1922.

ROBERT JOHN.